

## UNITED STATES PATENT OFFICE

2,182,135

## ALLOY STEEL

Gustav A. Reinhardt, Youngstown, Ohio, assignor to The Youngstown Sheet and Tube Company, Youngstown, Ohio, a corporation of Ohio

No Drawing. Application February 12, 1937,  
Serial No. 125,425

## 3 Claims. (Cl. 75—125)

This steel falls within that group of steels containing carbon, manganese, nickel and copper which have appreciably greater tensile strength and resistance to corrosion than ordinary steels 5 of similar carbon content and is characterized by properties which permit it to be readily and satisfactorily welded either electrically or by other usual methods. It is therefore particularly valuable for conditions of use in which a strong relatively non-corrodible steel of good weldability is desirable, especially as it readily lends itself to the usual manufacturing operations such as rolling, forging or the like.

I am aware that because of their strength and 15 corrosion resistant properties steels of this general group, particularly those containing chromium, have been widely used for many purposes, but as far as I have been able to ascertain these steels do not readily submit to welding and may 20 therefore be considered as of low or poor weldability as after welding they have a tendency to crack either in or adjacent the weld. In an effort to overcome this tendency it is therefore the usual practice to heat the part or parts just 25 prior to welding to about 150° F. or more over the entire area within a foot or so of the intended seam and, after formation of the weld, to subject this area as well as the weld itself to a heat treatment commonly known as a "stress relieving 30 treatment". This practice necessarily involves considerable expense and loss of time, while frequently because of the size or location of the parts or for other reasons the heat treatments either 35 cannot be performed at all or can be performed only with difficulty, so that in such instances the poor weldability of the steel makes it virtually impossible to turn out a satisfactory welded job irrespective of its cost.

The principal object of the invention therefore 40 is the provision of an alloy steel having good rolling and forging qualities, good weldability and greater corrosion resistance and strength than ordinary carbon steels of similar carbon content.

A further object of the invention is the provision 45 of an alloy steel of the copper-nickel group which can be welded by any of the methods of welding commonly in use without the necessity for preliminary or subsequent heat treatments of the work designed to obviate or minimize cracking in or in the vicinity of the weld.

Other objects, purposes and advantages of the 50 invention will hereafter more fully appear from the following description during which reference will be made by way of example to certain alloys of specific compositions, it being understood,

however, that these examples are to be considered as illustrative only since the invention in reality comprehends a new composition of matter in which the proportions of the ingredients are capable, within limits, of considerable variation 5 without affecting its predominant physical characteristics.

In addition to iron the steel or my invention contains carbon, silicon, nickel and copper, and my investigations indicate the proportions of 10 these elements should be preferably confined within the following limits:

|         | Per cent     |
|---------|--------------|
| Carbon  | 0.00—0.20    |
| Silicon | 0.10—0.25 15 |
| Copper  | 0.90—1.10    |
| Nickel  | 1.80—2.20    |

It may also be desirable, depending to some extent upon the purpose for which the steel is to be 20 used, to include in it sulphur up to 0.10% since its presence enhances machineability. Furthermore if it is desired to enhance the hardness and brittleness of the steel a small percentage of phosphorus may be included without materially 25 affecting its qualities in other respects.

The steel may also contain manganese in an amount requisite to maintain suitable malleability, ductility, rolling and other generally similar properties, but not in excess of 0.70% although at 30 least about 0.35% of this element may advantageously be present.

Several other elements which are customarily found in many kinds of steel may incidentally occur in very small quantities and are not appreciably inimical, but it is preferable that chromium and tungsten be wholly absent and that 35 boron, molybdenum, tantalum, uranium and vanadium be kept as low as possible since the presence of any of these in appreciable amounts 40 may impair the characteristics of the steel; however, a trace of aluminum resulting from this metal being used for "killing" the steel during or after pouring, or from other causes, is not particularly inimical.

When the ratio of nickel to copper is maintained at approximately 2:1 within the limits stated and the other elements named kept within the range hereinabove set forth, the resultant 50 alloy steel possesses corrosion resistant qualities in a ratio of 5:1 and strength in a ratio of 1.5:1 as compared to ordinary carbon steels of like carbon content, while its weldability is distinctly better than that of any other steels of the copper-nickel group of which I am aware. 55

Within or substantially within the foregoing range of permissive analyses for carbon, manganese, silicon, copper and nickel, a large number of alloy steels may be made, each differing in 5 specific analysis and perhaps slightly in other respects from the others yet each of good weldability, great strength and high-corrosion resistance, qualities not concurrently found in such other steels of the copper-nickel group.

10 Thus, two desirable compositions within the range mentioned contain:

|                                                      | I                     | II                    |
|------------------------------------------------------|-----------------------|-----------------------|
| 15 Carbon.....                                       | Percent<br>0.06- 0.68 | Percent<br>0.16- 0.20 |
| Manganese.....                                       | 0.35- 0.50            | 0.50- 0.65            |
| Sulphur.....                                         | 0.00- 0.035           | 0.00- 0.035           |
| Silicon.....                                         | 0.12- 0.20            | 0.12- 0.20            |
| Nickel.....                                          | 1.90- 2.10            | 1.90- 2.10            |
| Copper.....                                          | 0.95- 1.05            | 0.95- 1.05            |
| 20 Iron, including impurities in minute amounts..... | 96.62- 96.035         | 96.37- 95.765         |
|                                                      | 100.00 100.00         | 100.00 100.00         |

25 In view of the desirability of maintaining the steel free or substantially free from the several "rare" elements as above stated, namely chromium, tungsten, boron, molybdenum, tantalum, uranium and vanadium, it is usually preferable 30 in its production to avoid, in making up the furnace charge, the use of materials such as tool or alloy steel scrap or the like which frequently contain one or more of them, as by thus preventing their initial introduction into the charge 35 the necessity for subsequently endeavoring to reduce them in amount or remove them entirely is avoided.

It is believed the good weldability of this steel may be due in large measure to its low heat conductivity which is appreciably less than ordinary carbon steels, and which probably tends to prevent rapid dissemination of the heat from the weld into adjacent parts of the work and resultant too rapid cooling of the welded seam and metal in its vicinity with consequent minimization of internal stress necessitating, in other 45 steels, the stress relieving heat treatments to which reference has been made.

When rolled into sheets, plates or other shapes, 50 or forged or otherwise converted into finished or semi-finished articles of commerce the alloy can be readily welded by usual methods without the necessity of preheating in the vicinity of the weld and/or subjecting the welded article to subsequent stress relieving treatment as it 55 exhibits no material tendency to crack either in

the weld or in its vicinity while the weld is being made or after its completion, a characteristic or quality which I believe to be distinctly novel and unique in copper-nickel steel.

I am aware that certain steels have heretofore been suggested having good weldability but these steels do not possess other properties found in my alloy steel and thus are not, for example, comparable thereto in their strength and 10 resistance to corrosion. On the other hand, as far as is known to me, the other low alloy steels containing chromium and metals of that group which possess great strength and high resistance to corrosion are subject to cracking when an effort is made to weld them without preheat- 15 ing and subjection to a stress relieving treatment after the making of the weld. My alloy steel thus not only possesses desirable qualities of both of these two types of steels but is devoid of certain undesirable qualities inherent in each 20 of them.

It is thus characterized particularly by its good weldability in conjunction with relatively great strength and resistance to corrosion, while through avoidance of the use of large quantities of the more expensive alloying elements, its cost is maintained sufficiently low to permit its satisfactory commercial production and employment for many purposes.

Having thus described my invention, I claim 30 and desire to protect by Letters Patent of the United States:

1. An alloy steel comprising carbon not exceeding 0.20%, manganese 0.35% to 0.70%, copper 0.90% to 1.10%, nickel 1.80% to 2.20%, silicon 0.10% to 0.25%, sulphur not exceeding 0.10%, and substantially iron to make 100%, the ratio between the copper and nickel being as near as may be to 1:2.

2. An alloy steel comprising carbon 0.06% to 0.08%, manganese 0.35% to 0.50%, copper 0.95% to 1.05%, nickel 1.90% to 2.10%, silicon 0.12% to 0.20%, sulphur not exceeding 0.035%, and the remainder substantially iron to make 100%, the ratio between the copper and nickel being as near as may be to 1:2.

3. An alloy steel comprising carbon 0.16% to 0.20%, manganese 0.50% to 0.65%, copper 0.95% to 1.05%, nickel 1.90% to 2.10%, silicon 0.12% to 0.20%, sulphur not exceeding 0.035%, and the remainder substantially iron to make 100%, the ratio between the copper and nickel being as near as may be to 1:2.

GUSTAV A. REINHARDT. 55